# EUROPEAN PATENT SPECIFICATION

(11) **EP 1 913 196 B1**
(45) Date of publication and mention of the grant of the patent: **25.07.2018**
(21) Application number: 06756266.0
(22) Date of filing: 27.06.2006
(51) Int. Cl.: D06P 1/22, D06P 1/655, D06P 3/14, D06M 13/463, D06M 101/12

(54) **A PROCESS FOR DYEING OF WOOL OR SILK AND THEIR BLENDS (FIBRE /YARN/FABRIC) WITH INDIGO**
VERFAHREN ZUM FÄRBEN VON WOLLE ODER SEIDE UND IHREN MISCHUNGEN (FASER/GARN/FLÄCHENGEBILDE) MIT INDIGO
PROCEDE DESTINE A COLORER DE LA LAINE OU DE LA SOIE ET LEURS MELANGES (FIBRE/FIL/ETOFFE) AVEC DE L'INDIGO

(30) Priority: 28.06.2005 IN DE16742005
(43) Date of publication of application: 23.04.2008
(73) Proprietor: Malwa Industries Limited, Ludhiana 141 003, Punjab (IN)
(72) Inventor: OSWAL, Jangi Lal,Malwa Industries Limited, Ludhiana 141 003,Punjab (IN); OSWAL, Rishi Malwa Industries Limited, Ludhiana 141 003,Punjab (IN)
(74) Representative: Mitchell, Simon James
(86) International application number: PCT/IN2006/000216
(87) International publication number: WO 2007/000775

(56) References cited:
- GB-A- 294 890
- GB-A- 372 325
- GB-A- 448 272
- JP-A- 2004 210 887
- KR-A- 20040 043 873
- US-A- 2 254 965
- US-A- 4 615 709
- US-A- 4 742 589

## Description

### FIELD OF INVENTION

This invention relates to a process for dyeing of wool, silk or their blends (fibre/yarn/fabric) in tandem with indigo. In particular, this invention relates to a pretreatment of wool, silk or their blends in order to render it receptive to indigo dyeing.

### BACKGROUND OF THE INVENTION

The literature on wool discloses that the molecular grid of wool (Keratin) consists of polypeptide chains bound together by salt linkages and the covalent disulphide (-S-S) linkages. Such a literature further discloses that the disulphide bond is easily and readily degraded in the presence of alkali. Alkali disrupts the disulphide bonds and the fission of disulphide bonds results in the formation of thiol groups, which are very labile.
It is known that as a natural polyamide or polypeptide, silk Fibroin (degummed silk) exhibits free amino, carboxyl and phenolic substitutes with accessible hydroxyl groups. Silk and wool have a slightly cationic character with an isoelectric point at about pH 5.0. Thus, in an acidic solution, silk fibroin or wool takes on a positive charge through absorption of hydrogen ions. The resulting electric charge can be counter balanced with negatively charged anions of the dye, whilst dyeing with anionic dyes such as acid, metal complex, direct and reactive dyes.

It is known that indigo dyeing is carried out under highly alkaline pH values and that leuco indigo has an anionic charge. However, silk and wool have a tendency to lose their cationic property in presence of alkali. Both fibre and the dye being anionic under alkaline conditions, the net result is loss of dye-fibre affinity, lighter dyeing and poor fastness.

Two of the silk properties that determine its colour behaviour are, firstly, very fine fibre fibrils and, secondly high fiber orientation. These fine fibrils produce a large fiber surface. Such a large fiber surface results in the colour yield being very low and about twice as much dye is required for achieving a given dark shade. Further, the fastness is poor. A large fiber surface also leads to a high dye-strike rate even at very low temperature resulting into rapid saturation at the fiber surface and unlevel dyeing. The high orientation of the fibres, which is a barrier to diffusion, causes a very slow rate of further dye absorption, after the first rapid saturation.

Further, the surface of silk is very easily chafed by abrasion particularly when the material is in wet swollen state.

The polypeptide chains of silk fibroin may hydrolyze in boiling water or in steam. This becomes critical in the presence of acids or alkalis. Higher concentrations of alkalis rapidly dissolve silk and wool. Degradation of silk and wool is determined by pH and the type of alkali. The mechanical stress leads to splicing of silk threads, which is severe and irreparable damage.

Thus, it would be apparent that the normal known steps of dyeing of silk cannot be employed for indigo dyeing of silk (and wool) in general. Firstly, indigo dyeing is conventionally carried out under highly alkaline pH values. Both silk and wool would cease to be cationic under alkaline conditions and would assume anionic character losing electrostatic affinity for anionic leuco indigo. The result would be lighter and skittery dyeing and poor fastness.

The rope/slasher indigo dyeing machine is a long battery of several dip-squeeze-air modules with pre-wet, Pre-wet washes and post-dye-wash off boxes. The yarn passage through the said machine would be as long as 400-500 mtrs. At dyeing speed of for example 18-20 mtrs/minute, the yarn runs through hostile environment; for 25 minutes including long exposure to caustic soda, hot washes and mechanical stresses. All these could deteriorate the mechanical properties of silk and wool.

GB 448,272 discloses a process for dyeing fibrous materials suitable for the textile industry with vat dyestuffs consisting of pre-treating the fibrous material with quaternary ammonium compounds.

GB 372,325 discloses a process for improving the softness or purity of fibrous materials such as textiles by treatment with aqueous solutions of amines or ammonium bases which contain at least one alkyl or cycloalkyl radical with at least eight carbon atoms, or water-soluble salts of the bases.

US 2,254,965 discloses a process for dyeing fibrous materials.

US 4,615,709 discloses cationic compounds used for improving the dyeing properties of a textile material by treating the textile material before or after dyeing with an anionic dye.

### OBJECTS OF THE INVENTION

An object of this invention is to propose a novel process for the dyeing of wool, silk or blends thereof with indigo in conventional dyeing machines.

Yet another object of this invention is to propose a novel pretreatment process for dyeing of wool, silk or blends thereof with indigo.

Still another object of this invention is to propose a novel process for the dyeing of wool, silk or blends thereof with indigo, which reduces the severity of dyeing conditions.

A further object of this invention is to propose a novel process for the dyeing of wool, silk or blends thereof with indigo, which avoids any damage being caused to wool or silk.

A still further object of this invention is to propose a novel process for the dyeing of wool, silk or blends thereof with indigo, which provides a dark and level indigo shade.

Yet further object of this invention is to propose a novel process for the dyeing of wool, silk or blends thereof with indigo, which provides adequate fastness.

Still a further object of this invention is to propose a novel process for the dyeing of wool or silk or blends thereof with indigo, which is efficient.

### DESCRIPTION OF THE INVENTION

It is known that alkali disrupts the disulphide bonds in wool and results in the formation of thiol groups. Such a reaction is utilized in the present invention in that before the labile thiol groups recombine or form fresh cross links, the thiol groups are, in situ, brought in contact with (leuco) indigo, some hydrogen bonds/salt linkages between the dye and the thiol groups in the substrate are effected. Thus, the total dye-combining capacity of the substrate is increased by generating additional dye-combining groups or sites by the action of alkali on wool. The rate and extent of dye absorption is enhanced by virtue of increased accessibility of the fibre to the dye.

In accordance with this invention, a mordanting of wool and silk in the form of cationization on line enhances dye-fibre affinity by virtue of imparted cationic dye-combining sites for indigo which is anionic in alkaline media. Such mordanting also reduces the heterogeneity in the substrate and offer thereby level dyeing.

Wool and silk are sensitive to alkali and might degrade significantly when in contact with alkali particularly caustic soda for any appreciable length of time. In case of wool, such a normally negative point is instead taken advantage of by using generated thiol groups as additional dye combining sites.

Thus, to overcome the disadvantages of the prior art, cationization of wool and silk or deposition of insitu generated cationic polymer/oligomer within fibre provides the required result in that the cationic charge in the substrate could attract the anionic leuco indigo dye

According to this invention there is provided a process for the pretreatment of wool, silk or blends thereof comprising the step of online cationization of silk, wool or blends thereof to render it receptive to indigo dyeing by imparting a cationic charge and generating dye-combining sites.

Thus, the invention provides a process for the on-line pre-treatment of a substrate comprising wool, silk or blends thereof rendering the substrate receptive for a subsequent step of indigo dyeing, the pre-treatment step comprising generating dye combining sites by: (i) cationisation on the substrate; and (ii) treatment with caustic soda; for a period sufficient to generate said sites, wherein pre-treatment step (i) includes the step of cationising the substrate by passing the substrate through a pre-treatment bath containing a cationising compound solution followed by aeration such that the cationising compound can penetrate into the substrate, and wherein the pre-treatment step is carried out for 5 to 30 seconds and the aeration is carried out for 30 to 180 seconds. The treatment comprises in the step of cationization by passing wool, silk or blends thereof through pre-treatment baths and then subjecting to the step of a passage in air, which is online. The online pre-treatment could be effected either at ambient temperature or at subambient temperature, for example, at 12-15°C. The pre-treatment bath comprises 3- to 120 gpl, and preferably 3 to 80 gpl of cationizing compound and 3 to 25 gpl of caustic soda either separately or in admixture.
Reference is now made to the step of dyeing of silk or wool with indigo subsequent to the pretreatment step in a manner known in the art, but the step of dyeing comprises in passing in tandem the pretreated silk, wool or blend through a plurality of indigo dye baths following the dip-squeeze-air (oxidation) steps.
In accordance with this invention, the dye bath contains (leuco) indigo, soda ash sodium hydroxide, sodium hydrosulphite and
known chemical auxiliaries. As described hereinabove, wool and silk have a tendency to lose its cationic charge in the presence of alkali. Simultaneously, the addition of alkali to the dye bath is necessary in order to render the dye soluble. However, the pretreatment step renders silk or wool receptive to anionic leuco dye by virtue of imparted cationization and generated dye combining sites in the substrate. Thus, each dye bath contains 1.0 to 3.5 gpl indigo and upto 8 dye baths may be provided. The passage of wool or silk through each dye bath is for a period of 5 to 30 seconds each followed by the step of squeez and oxidation for a period of 30 to 180 seconds for each step of oxidation. The dye-bath recipe contains soda ash mostly and between 15-20 gp1, in place of caustic soda. The latter is used for fine tuning of dye bath pH. The caustic soda and the cationizing chemical in the pre-treatment are kept at subambient treatment in accordance with on embodiment of this invention. This is to reduce the severity of the process and help substrate retain its original strength.

Reference is made to the online pretreatment step in distinction to a batch process. One of the aspects of the present invention resides in the online pretreatment step which provides a short period of contact of wool, silk of its blends with caustic soda and cationizing chemicals. It is known that wool, silk or its blend is sensitive to caustic soda. Thus, one of the aspects of the present invention is to ensure that the wool, silk or its blends is not deteriorated or damaged by the pretreatment step, which is ensured by a reduced contact period with the cationizing chemicals by such an online step.

### EXAMPLE

The wool yarn was subjected to online cationization. The original sample as well as the cationized sample were then analyzed for their nitrogen contents by Kjeldahl method. The sample showed increase in nitrogen content over the control by 0.35%.
The nitrogen content of the cationizing chemical viz., 3-chloro-2-hydroxy propyl trimethyl ammonium chloride is 9.18%.

The 0.35% increase in nitrogen content in cationized sample would therefore mean 5.8 gram of cationizing chemical was added up to 100 grams of wool.

The spectral study indicated no major change in the structural pattern of wool.

The nitrogen increase in case of silk was 0.2% which means 3.3 gms of cationizing chemical was deposited onto 100 gms of silk.

### DESCRIPTION WITH REFERENCE TO ACCOMPANYING DRAWING

Reference is made to fig. 1 of the accompanying drawing which illustrates a schematic line diagram of a known rope dyeing apparatus but modified to contain the pretreatment steps.

As shown in fig. 1, the pretreatment apparatus contains Box 1 and Box 2 with squeeze rollers SR1 therebetween.

First box Box 1 may contain cationizing chemical solution followed by aeration thereafter which allows time for cationizing chemical to penetrate well into wool/silk substrate.

The second box Box 2 may contain caustic soda solution also followed by aeration.

Aeration allows time for reaction between wool/silk and cationizing chemical in the presence of caustic soda. Alternatively, Box 1 may contain both cationizing chemicals and caustic soda.

After impregnation of wool/silk with the said cationizing chemical, an aeration is effected which allows for the time for the reaction between wool/silk and cationizing chemical in the presence of caustic soda.

The second box Box 2 in such an instance could be empty-or could be used for a water-rinse

Indigo dyeing then follow in tandem, with conventional and known steps of indigo dyeing, viz., dip-squeeze-air.
As shown in fig. 1, the pretreated substrate then passes through a plurality of dye boxes, for example 1 to 8 dye boxes, followed each time by aeration. The substrate is then subjected to post dyeing wash off in wash boxes and then passed through drying cans.

## Claims

1. A process for the on-line pre-treatment of a substrate comprising wool, silk or blends thereof rendering the substrate receptive for a subsequent step of indigo dyeing, the pre-treatment step comprising generating dye combining sites by:
(i) cationisation on the substrate; and
(ii) treatment with caustic soda;
for a period sufficient to generate said sites,
wherein pre-treatment step (i) includes the step of cationising the substrate by passing the substrate through a pre-treatment bath containing a cationising compound solution followed by aeration such that the cationising compound can penetrate into the substrate, and
wherein the pre-treatment step is carried out for 5 to 30 seconds and the aeration is carried out for 30 to 180 seconds.

2. The process according to claim 1, wherein the pre-treatment bath comprises 3 to 80 grams/litre of cationising compound and 3 to 25 grams/litre of caustic soda.

3. The process according to claim 1, wherein the pre-treatment step is carried out at ambient temperature.

4. The process according to claim 1 or claim 2, wherein the pre-treatment step is carried out at 12 to 15°C.

5. The process according to claim 1, wherein the cationising compound comprises 3-chloro-2-hydroxypropyl trimethyl ammonium chloride.

## Patentansprüche

1. Verfahren zur On-Line-Vorbehandlung eines Substrats, das Wolle, Seide oder Gemische davon umfasst, wodurch das Substrat für einen anschließenden Schritt des Indigofärbens empfänglich gemacht wird, wobei der Vorbehandlungsschritt das Erzeugen von Farbstoffkombinationsstellen durch:
(i) Kationisierung auf dem Substrat und
(ii) Behandlung mit Ätznatron
für einen Zeitraum, der dazu ausreicht, die Stellen zu erzeugen, umfasst,
wobei der Vorbehandlungsschritt (i) den Schritt des Kationisierens des Substrats durch Leiten des Substrats durch ein Vorbehandlungsbad, das eine kationisierende Verbindungslösung enthält, gefolgt von Belüften, so dass die kationisierende Verbindung in das Substrat eindringen kann, beinhaltet und
wobei der Vorbehandlungsschritt für 5 bis 30 Sekunden durchgeführt wird und das Belüften für 30 bis 180 Sekunden durchgeführt wird.

2. Verfahren nach Anspruch 1, wobei das Vorbehandlungsbad 3 bis 80 Gramm/Liter kationisierende Verbindung und 3 bis 25 Gramm/Liter Ätznatron umfasst.

3. Verfahren nach Anspruch 1, wobei der Vorbehandlungsschritt bei Umgebungstemperatur durchgeführt wird.

4. Verfahren nach Anspruch 1 oder 2, wobei der Vorbehandlungsschritt bei 12 bis 15 °C durchgeführt wird.

5. Verfahren nach Anspruch 1, wobei die kationisierende Verbindung 3-Chlor-2-hydroxypropyltrimethylammoniumchlorid umfasst.

## Revendications

1. Procédé pour le prétraitement en ligne d'un substrat comprenant de la laine, de la soie ou des mélanges de celles-ci sensibilisant le substrat pour une étape subséquente de teinture à l'indigo, l'étape de prétraitement comprenant la production de sites de combinaison de colorant par :
(i)cationisation sur le substrat ; et
(ii) traitement avec de la soude caustique ;
pendant une durée suffisante pour produire lesdits sites,
dans lequel l'étape de prétraitement (i) comprend l'étape de cationisation du substrat par passage du substrat dans un bain de prétraitement contenant une solution de composé de cationisation suivi d'une aération de façon telle que le composé de cationisation peut pénétrer dans le substrat et
dans lequel l'étape de prétraitement est effectuée pendant 5 à 30 secondes et l'aération est effectuée pendant 30 à 180 secondes.

2. Procédé selon la revendication 1, dans lequel le bain de prétraitement comprend 3 à 80 grammes/litre de composé de cationisation et 3 à 25 grammes/litre de soude caustique.

3. Procédé selon la revendication 1, dans lequel l'étape de prétraitement est effectuée à température ambiante.

4. Procédé selon la revendication 1 ou la revendication 2, dans lequel l'étape de prétraitement est effectuée à 12 à 15 °C.

5. Procédé selon la revendication 1, dans lequel le composé de cationisation comprend du chlorure de 3-chloro-2-hydroxypropyltriméthylammonium.
